# EUROPEAN PATENT SPECIFICATION

(11) **EP 1 609 618 B1**
(45) Date of publication and mention of the grant of the patent: **26.03.2008**
(21) Application number: 04707676.5
(22) Date of filing: 03.02.2004
(51) Int. Cl.: B41C 1/10, G03F 7/36, B41N 1/14

(54) **LITHOGRAPHIC PRINTING PLATE ORIGINAL FORM AND PLATE MAKING METHOD**
AUSGANGSFORM FÜR LITHOGRAPHISCHE DRUCKPLATTE UND PLATTENHERSTELLUNGSVERFAHREN
FORME INITIALE DE PLAQUE D'IMPRESSION LITHOGRAPHIQUE ET PROCEDE DE FABRICATION DE PLAQUE ASSOCIE

(30) Priority: 04.02.2003 JP 2003027067
(43) Date of publication of application: 28.12.2005
(73) Proprietor: Kodak Polychrome Graphics Japan Ltd., Tokyo (JP)
(72) Inventor: HAYASHI, K., Kodak Polychr.Graphics,Japan Ltd., Oura-gun, Gunma 370-0723 (JP)
(74) Representative: Haile, Helen Cynthia
(86) International application number: PCT/JP2004/001033
(87) International publication number: WO 2004/069552

(56) References cited:
- JP-A- 11 028 871
- JP-A- 2000 250 202
- JP-A- 2000 263 958
- JP-A- 2001 001 661
- JP-A- 2001 228 602
- JP-A- 2001 296 669
- JP-A- 2003 025 531
- JP-A- 2004 090 438

## Description

### Technical field

The present invention pertains to a lithographic printing plate original and a plate manufacturing method. In particular, the present invention pertains to lithographic printing plate original, which can be directly manufactured by irradiating an IR laser beam based on digital signals and can be directly loaded into a printer without performing development after exposure, and to a plate manufacturing method.

### Background technology

In recent years, in company with the progress made in computer image processing technology, a method of directly writing an image by means of light irradiation corresponding to digital signals has been developed. The computer to plate (CTP) system, which applies the aforementioned method to a lithographic printing plate in order to directly form an image on the lithographic printing plate original without performing output to a silver salt mask film, has attracted a lot of attention. A CTP system using infrared radiation, or on high output laser with maximum strength in the IR region, as the light source of light irradiation makes it possible to obtain a high resolution image with a short period of exposure, and allows processing of the lithographic printing plate used in that system in a bright room. In particular, a solid-state laser and a semiconductor laser that emit IR radiation with a wavelength in the range of 760-1200 nm is desired, since it has small size and high output, and can be obtained easily.

Japanese Kokai Patent Application No. Hei 11 [1999]-202481 disclosed a positive lithographic printing plate original that can form images by performing development using a developer after the solid-state laser or semiconductor laser that emits said IR radiation is used to perform exposure. It has a photosensitive layer made of a positive photosensitive composition containing an alkali soluble resin (novolac resin, etc.), a light-heat converting agent (dye, pigment, or other IR absorbent), and a compound that can crosslink the alkali soluble resin under thermal effect.

Recently, in order to simplify the plate manufacturing operation, improve the operational environment at the plate manufacturing site, and protect the environment, there is a demand for a lithographic printing plate original that can be directly loaded into a printer after exposure without performing development using a developer containing an organic solvent or alkaline substance. However, since the positive photosensitive composition disclosed in Japanese Kokai Patent Application No. Hei 11 [ 1999]-202481 contains novolac resin or another alkaline soluble resin as the binder resin, the photosensitive lithographic printing plate with a photosensitive layer made of the aforementioned composition requires development processing using a strong alkaline developer.

Japanese Kokai Patent Application No. Hei 6[1994]-43634, Hei 11[1999]-65106, 2000-211097, Japanese Kohyo Patent No. 2002-500973 disclosed lithographic printing plate originals that require no development after exposure. After an IR laser beam is irradiated on the image forming layer of the lithographic printing plate original, images can be formed by eliminating the image forming layer in the irradiated part (ablation).

The image forming element described in Japanese Kokai Patent Application No. Hei 6[1994]-43635 has an image forming layer containing a polymer with azido groups in a side chain, formed on a base material. In this image forming element, images can be formed when the azido groups in the exposed part are decomposed as a result of exposure to eliminate the image forming layer. However, since the decomposable azido groups are in the side chain of the polymer, it is difficult to decompose and eliminate the polymer by means of exposure. The ablation efficiency (sensitivity) is poor.

For the lithographic printing plate original disclosed in Japanese Kokai Patent Application No. Hei 11 [ 1999]-65106, an image forming layer with a specific polyazo compound held by a binder resin is formed on an aluminum support. In this lithographic printing plate original, images can be formed when the polyazo compound in the exposed part is decomposed as a result of exposure to eliminate the image forming layer. However, the polyazo compound has a low molecular weight. The image forming layer containing such compound has weak resistance to wear and tear, and the durability of the lithographic printing plate is not good enough. Also, since the polyazo compound is insoluble in organic solvent, it must be dispersed and coated in order to form the image forming layer on the support. This results in poor productivity.

The printing material disclosed in Japanese Kokai Patent Application No. 2000-211097 has a first imaging layer, a second imaging layer, and a top layer on a substrate. The polymer of the second imaging layer has functional groups and azo groups. For this printing material, the azo groups in the exposed part are decomposed as a result of exposure to generate gas. Images can be formed when the imaging layer is destroyed by the bubbles of this gas and the top layer is peeled off. However, since this printing material has multiple layers with different compositions laminated on a substrate, peeling tends to occur on the boundary surface of each layer. As a result, the durability is poor.

Japanese Unexamined Patent Application 11-028871 describes a direct write type element having a heat-sensitive layer under a top silicone rubber layer. Nitrogen-containing compounds are avoided. The substrate is a degreased aluminum sheet.

The lithographic printing plate disclosed in Japanese Kohyo Patent No. 2002-500973 has an ablation-absorptive layer formed on a support base material. For this lithographic printing plate, images can be formed when the ablation-absorptive layer in the exposed part is removed by means of exposure. However, since the polymer of the ablation-absorptive layer has no pyrolytic group, it is difficult to decompose and eliminate the polymer by means of exposure. Therefore the sensitivity is not high enough.

The purpose of the present invention is to provide a lithographic printing plate original, which can be directly manufactured by irradiating an IR laser beam based on digital signals and can be directly loaded into a printer without performing development after exposure, and has good ablation efficiency (sensitivity) as well as excellent durability of the lithographic printing plate obtained.

### Disclosure of the invention

The lithographic printing plate original of the present invention is characterized by the fact that the lithographic printing plate original has a support having a hydrophilic surface and a lipophilic layer formed on the support, and the lipophilic layer contains a crosslinked product formed by crosslinking a polymer having a pyrolytic group in the main chain with a crosslinking agent, the pyrolytic group being an azo, diazo, hydrazide, nitro, ammonium or other ammonium salt.

The lithographic printing plate original can be manufactured directly by irradiating an IR laser beam based on digital signals. The manufactured plate can be loaded into a printer directly without performing development after exposure. The ablation efficiency (sensitivity) is good, and the lithographic printing plate obtained has excellent durability.

In this case, if the aforementioned pyrolytic group is an azo group, the ablation efficiency (sensitivity) can be further improved.

Also, if the aforementioned polymer has functional groups that can react with the crosslinking agent, the durability of the lithographic printing plate obtained can be further improved.

Because the aforementioned support has a hydrophilic surface, the hydrophilicity of the non-scanning part of the lithographic printing plate obtained can be further improved.

If the aforementioned lipophilic layer contains a light-heat converting substance, the ablation efficiency (sensitivity) can be further improved.

If there is a hydrophilic layer between the aforementioned support and the lipophilic layer, a good lithographic printing plate without printing stain can be obtained.

If the aforementioned hydrophilic layer contains a light-heat converting substance, the ablation efficiency (sensitivity) can be further improved.

Also, the plate manufacturing method of the present invention is characterized by the fact that the lithographic printing plate original of the present invention is exposed using an IR laser beam to eliminate the lipophilic layer in the exposed part.

### Brief explanation of figures

Figure 1 is a schematic cross-sectional view illustrating an example of the lithographic printing plate original disclosed in the present invention.
Figure 2 is a schematic cross-sectional view illustrating another example of the lithographic printing plate original disclosed in the present invention.

### Best embodiment of the invention

In the following, the present invention will be explained in more detail.

Figure 1 is a schematic cross-sectional view illustrating an example of the lithographic printing plate original disclosed in the present invention. This lithographic printing plate original has a support 11, and a lipophilic layer 12 formed on support 11.

### <Support>

The support can be made of aluminum, zinc, copper, stainless steel, iron, or other metal sheet; polyethylene terephthalate, polycarbonate, polyvinyl acetal, polyethylene, or other plastic film; paper whereon a synthetic resin is melted and coated or a synthetic resin solution is coated, composite material obtained by forming a metal layer on a plastic film by means of vacuum deposition or lamination; or other material that can be used for the support of a lithographic printing plate. Among these materials, it is preferred to use aluminum or an aluminum coated composite support.

In order to improve water retention property and adhesion to the photosensitive layer, the surface of the support is processed into a hydrophilic surface. Said surface processing includes the brush polishing method, ball polishing method, electrolytic etching, chemical etching, liquid honing, sand blasting, or other surface roughening processes, and combinations of them. It is particularly preferred to perform a surface roughening processing in which electrolytic etching is involved.

An acid, alkali, or aqueous solution containing their salt, or an aqueous solution containing an organic solvent, is used as the electrolytic bath during electrolytic etching.

If necessary, the aluminum support with the roughened surface is dematted using an aqueous solution of acid or alkali. It is preferred to apply anode oxidization to the aluminum support obtained. In particular, it is preferred to perform the anode oxidization in a bath containing sulfuric acid or phosphoric acid.

Also, if necessary, it is also possible to carry out silicate processing (sodium silicate, potassium silicate), potassium fluoride zirconate processing, phosphomolybdate processing, alkyl titanate processing, polyacrylic acid processing, polyvinyl sulfonic acid processing, phosphonic acid processing, phytic acid processing, processing using a salt of a hydrophilic organic polymeric compound and a bivalence metal, hydrophilic processing using an undercoat of a water soluble polymer with sulfonic acid groups, color processing using acidic dyes, or silicate electroplating, etc.

After the surface roughening processing (sand processing) and the anode oxidization, it is preferred to apply hole sealing processing to the aluminum support. The hold sealing processing can be carried out by immersing the aluminum support in hot water or a hot aqueous solution containing inorganic salt or organic salt, or by means of a steam bath.

### <Lipophilic layer>

The lithographic printing plate contains a crosslinked product formed by crosslinking a polymer with a pyrolytic group in the main chain with a crosslinking agent.

### (Polymer with a pyrolytic group in the main chain)

There is no special limitation on the polymer as long as it has a pyrolytic group in the main chain. Examples of such polymer include polyesters, polyurethanes, etc. having a pyrolytic group in the main chain. In this case, "having a pyrolytic group in the main chain" means that the pyrolytic group itself forms part of the main chain, or the pyrolytic group is directly bonded to the carbon atom, nitrogen atom, etc. in the main chain.

The polyester with a pyrolytic group in the main chain can be synthesized using the method of reacting a diol with a pyrolytic group with dicarboxylic acid, chloride dicarboxylate or the anhydride of tetracharboxylic acid, and, if necessary, other diols; or the method of reacting a diol with dicarboxylic acid, chloride dicarboxylate or the anhydride of tetracarboxylic acid with a pyrolytic group, and, if necessary, other dicarboxylic acid, chloride dicarboxylate or the anhydride of tetracarboxylic acid.

The polyurethane with a pyrolytic group in the main chain can be synthesized using the method of reacting a diol with a pyrolytic group with diisocyanate, and if necessary, other diols; or the method of reacting a diol with diisocyanate having a pyrolytic group, and if necessary, other diisocyanates.

When synthesizing the polyester or polyurethane with a pyrolytic group in the main chain, the molar ratio of the bifunctional compound with a pyrolytic group (diol, dicarboxylic acid, chloride dicarboxylate, tetracarboxylic acid, or diisocyanate with a pyrolytic group) and the other bifunctional compounds (diol, dicarboxylic acid, chloride dicarboxylate, tetracarboxylic acid, or diisocyanate with no pyrolytic group) is preferred to be in the range of 10:90 - 50:50. If the content of the bifunctional compound with a pyrolytic group is less than 10 mol%, the ablation efficiency (sensitivity) of the lithographic printing plate original obtained is not good enough.

The pyrolytic groups for use in the lithographic printing plate original are selected from the azo group (-N=N-), diazo group (=N₂), hydrazide group (-NH-NH-), nitro group (-NO2); ammonium group (-N⁺(R )z-), and other ammonium salts, etc. In this case, R represents a hydrogen atom or alkyl group, aryl group, or other hydrocarbon group. The pyrolytic group is preferred to be an azo group, ammonium group, or nitro group so that the main chain of the polymer can be cut off easily, and the lithographic printing plate original obtained has excellent ablation efficiency (sensitivity). An azo group is particularly preferred since gas can be generated during pyrolysis to accelerate the ablation.

The polymer with a pyrolytic group is preferred to have a functional group that can react with the crosslinking agent to be described later. Examples of the functional group include the hydroxyl group, carboxylic acid group, amino group, thiol group, etc. With the aforementioned functional group, the polymer with a pyrolytic group in the main chain and the crosslinking agent can form a crosslinked product with a strong crosslinked structure. As a result, the resistance to war of the lipophilic layer can be improved, and the durability of the lithographic printing plate obtained can be improved.

The mass average molecular weight of the polymer with a pyrolytic group in the main chain is preferred to be in the range of 2000-100000. If the mass average molecular weight of the polymer is smaller than 2000, the image part where the image is formed becomes weak, and the printing durability becomes poor. On the other hand, if the mass average molecular weight of the polymer exceeds 100000, dissolution in the coating solvent becomes difficult. As a result, the coating property becomes poor.

It is also possible to use a pyrolytic compound besides a polymer with a pyrolytic group in the main chain. Examples of pyrolytic compound that can be used include cyanoacrylate polymer, α-methyl styrene polymer, (meth)acrylate monomer polymer; polycarbonate, nitrocellulose, cellulose acetate butyrate, cellulose acetate, polyvinyl chloride, polyvinylidene chloride, polyvinyl pyrrolidone, polyorthoester, acrylonitrile polymer, polyamide, polyurethane, maleic acid resin, polythioacetone ammonium nitrate, potassium nitrate, sodium nitrate, and other nitro compounds, organic peroxides, azo compounds, diazo compounds, and hydrazine compounds, etc.

### (Crosslinking agent)

There is no special limitation on the crosslinking agent as long as it can crosslink the aforementioned polymer with a pyrolytic group in the main chain. Examples of the crosslinking agent include hexamethoxymethyl melamine, hexahydroxy methyl melamine, dihydroxymethyl urea, polyhydric ethylene imine, polyhydric epoxy compound, polyhydric oxazoline polymer, polyhydric carboxyimide polymer, polyisocyanate, polyhydric carboxylic anhydride, etc. Among them, hexamethoxy methyl melamine is preferred in order to obtain a crosslinked product with high crosslinking density, and to realize good stability in the coating solution.

The amount of the crosslinking agent is preferred to be in the range of 10-50 parts by mass with respect to 100 parts by mass of the polymer with a pyrolytic group in the main chain. If the amount of the crosslinking agent is less than 10 parts by mass with respect to 100 parts by mass of the polymer with a pyrolytic group in the main chain, the resistance to wear of the lipophilic layer becomes low, and the durability of the lithographic printing plate obtained is not good enough. If the amount of the crosslinking agent exceeds 50 parts by mass with respect to 100 parts by mass of the polymer with a pyrolytic group in the main chain, the lipophilic layer is difficult to remove under IR laser irradiation, and the ablation efficiency (sensitivity) becomes poor.

### (Crosslinked product)

The crosslinked product is obtained when the polymer with a pyrolytic group in the main chain is crosslinked by a crosslinking agent. It is the main component of the lipophilic layer.

To obtain the crosslinked product, for example, a coating solution prepared by dissolving the polymer with a pyrolytic group in the main chain and the crosslinking agent in a solvent is coated on a support, followed by drying. Under the heat of drying, the polymer with a pyrolytic group in the main chain reacts with the crosslinking agent to generate the crosslinked product. It is also possible to add a crosslink into the coating solution in order to accelerate the reaction between the polymer with a pyrolytic group in the main chain and the crosslinking agent.

### (Light-heat converting substance)

The lipophilic layer is preferred to contain a light-heat converting substance, which absorbs light to generate heat.

The light-heat converting substance can generate heat efficiently under IR laser irradiation to accelerate the ablation of the lipophilic layer. Various types of pigments or dyes can be used as this substance.

Commercially available pigments and the pigments described in the Color Index Handbook "The Newest Pigment Handbook", edited by the Japanese Pigment Technical Association, 1977, "The Newest Pigment Application Technology" (published by CMC, 1986), "Printing Ink Technology" (published by CMC, 1984), etc. Pigment types include black pigments, yellow pigments, orange pigments, brown pigments, red pigments, violet pigments, blue pigments, green pigments, fluorescent pigments, and other polymer composite pigments. More specifically, examples of the pigments that can be used include insoluble azo pigments, azo lake pigments, condensed azo pigments, phthalocyanine type pigments, anthraquinone type pigments, perillene and perinone pigments, thioindigo pigments, quinacridone type pigments, dioxazine type pigments, isoindolinone type pigments, quinophthalone type pigments, dyed lake pigments, azine pigments, nitroso pigments, nitro pigments, natural pigments, fluorescent pigments, inorganic pigments, carbon black, etc.

Among the aforementioned examples, carbon black is particularly preferred since it can absorb light from the near IR region to the IR region to efficiently generate heat, and has good cost effectiveness. Grafted carbon black having various types of functional groups and good dispersibility is marketed as this type of carbon black. Examples are described on p. 167 in "Carbon Black Handbook 3rd Edition" (edited by the Carbon Black Association, 1995), p. 111 of "Characteristics of Carbon Black and Optimum Composition and Application Technology" (Technical Information Association, 1997). These carbon blacks can all be used in the present invention.

The aforementioned pigments can be used directly without surface processing or after a well-known surface processing is performed. The well-known surface processing includes the method of surface coating with resin or wax, the method of attaching a surfactant, and the method of bonding a silane coupling agent or epoxy compound, polyisocyanate, or other reactive substance to the pigment surface. These surface processing methods are described in "Properties and Applications of Metallic Soap" (Sachi Bookstore), "Newest Pigment Application Technology" (published by CMC, 1986), "Printing Ink Technology" (published by CMC, 1984).

The particle size of the pigment used in the present invention is preferred to be in the range of 0.01-15 micrometers, more preferably, in the range of 0.01-5 micrometers.

Conventional dyes can be used in the present invention. Examples include those described in "Handbook of Dyes" (edited by the Organic Synthetic Chemistry Association, 1970), "Color Material Engineering Handbook" (edited by the Color Material Association, Asakura Bookstore, 1989), "Technology and Marketing of Industrial Coloring Materials" (CMC, 1983), "Chemistry Handbook, Application Chemistry chapter" (edited by the Japanese Chemistry Association, Maruyoshi Bookstore, 1986). More specifically, examples of the dyes that can be used in the present invention include azo dyes, metal chain salt azo dyes, pyrazolone azo dyes, anthraquinone dyes, phthalocyanine dyes, carbonium dyes, quinonimine dyes, methine dyes, cyanine dyes, indigo dyes, quinoline dyes, nitro dyes, xanthene dyes, thiazine dyes, azine dyes, oxazine dyes, etc. Among these dyes, those that can absorb light from the near IR region to the IR region are particularly preferred.

Examples of the dyes that can absorb light from the near IR region to the IR region include cyanine dyes, methine dyes, naphthoquinone dyes, squalium dyes, allyl benzo(thio)pyridium salts, trimethlyene thiapyrylium salt, pyrylium type compounds, pentamethylene thiopyrylium salt, IR absorptive dyes, etc.

At least one type of the aforementioned pigments or dyes, which can absorb the specific wavelength of the light source to be described later to generate heat, is selected and added into the aforementioned coating solution to be contained in the lipophilic layer. In particular, when a light-heat converting substance having a maximum absorption wavelength (λmax) from the near IR region to the IR region of 760-3000 nm, the photosensitive lithographic printing plate obtained can be handled in a bright room. This is more preferred.

The content of the light-heat converting substance in the lipophilic layer is preferred to be in the range of 0.5-70 mass%, more preferably, in the range of 1-50 mass%. If the content is less than 0.5 mass%, only a small quantity of heat will be generated. As a result, the ablation of the exposed part becomes insufficient. If the content is more than 70 mass%, the lipophilic layer is easy to damage, and stains tend to occur in the non-image part.

### (Other components)

If necessary, it is also possible to add conventional additives, such as coloring materials (dyes, pigments), surfactants, plasticizers, stabilizers, etc. into the lipophilic layer.

Preferred dyes include crystal violet, malachite green, Victoria blue, methlylene blue, ethyl violet, Rhodamine B, and other basic oil soluble dyes. Commercially available products include "Victoria Pure Blue BOH" (product of Hodogoya Chemical Industry Co., Ltd.), "Oil Blue #603" (product of Orient Chemical Industry Co., Ltd.), "VPB-Naps (naphthalene sulfonate of Victoria pure blue)" (product of Hodogoya Chemical Industry Co., Ltd.), "D11" (product of PCAS Corporation), etc. Examples of pigments include phthalocyanine blue, phthalocyanine green, dioxazine violet, quinacridone red, etc.

Examples of the surfactants include fluorine-based surfactants, silicone-based surfactants, etc.

Examples of plasticizers include diethyl phthalate, dibutyl phthalate, dioctyl phthalate, tributyl phosphate, trioctyl phosphate, tricresyl phosphate, tri(2-chloroethyl) phosphate, tributyl citrate, etc.

Examples of stabilizers include phosphoric acid, phosphorous acid, nitric acid, tartaric acid, malic acid, citric acid, dipicolinic acid, polyacrylic acid, benzene sulfonic acid, toluene sulfonic acid, etc.

Although the content of the various types of additives varies depending on the purpose, it is preferred to be in the range of 0-30 mass% in the lipophilic layer.

### <Hydrophilic layer>

As shown in Figure 2, the lithographic printing plate original of the present invention has hydrophilic layer 13 between support 11 and lipophilic layer 12. When said hydrophilic layer 13 is used, the remaining gas of lipophilic layer 12 left in the exposed part that is not eliminated under irradiation of the IR laser beam can be completely eliminated by the wetting water, printing ink, etc. used during printing. In other words, removal of lipophilic layer 12 under irradiation of the IR laser beam is easier when lipophilic layer 12 is in contact with hydrophilic layer 13 instead of support 11. Also, when hydrophilic layer 13 is used, it is difficult to cause heat damage to the surface of support 11 under irradiation of the IR laser beam.

Examples of the polymer that can be used to form the hydrophilic layer include polyvinyl alcohol (saponified polyvinyl acetate), polymer salt of carboxylic acid, carboxyl methyl cellulose salt, etc. Among them, polyvinyl alcohol is preferred because of its excellent resistance to wear.

In order to improve the resistance to wear, it is also possible to add organic aluminum chelate compound, organic titanium chelate compound, or organic zirconium chelate compound into the hydrophilic layer. Among them, the organic aluminum chelate compound is preferred because of its excellent stability in the coating solution. An example of the organic aluminum chelate compound is Alcatic AL-135 produced by Matsumoto Pharmaceutical Industrial Co., Ltd.

The amount of organic aluminum chelate compound is preferred to be in the range of 20-150 parts by mass with respect to 100 parts by mass of the polymer that forms the hydrophilic layer. If the amount of the organic aluminum chelate compound is less than 20 parts by mass with respect to 100 parts by mass of the polymer that forms the hydrophilic layer, the crosslinked structure is not good enogh, and the resistance to wear of the hydrophilic layer cannot be improved. If the amount of the organic aluminum chelate compound exceeds 150 parts by mass with respect to 100 parts by mass of the polymer that forms the hydrophilic layer, the hydrophilic layer may have not sufficient hydrophilicity.

The hydrophilic layer may also contain the aforementioned light-heat converting substance in order to further improve the ablation effect.

The content of the light-heat converting substance in the hydrophilic layer is preferred to be in the range of 0.1-10 mass%, more preferably in the range of 1-5 mass%. If the content is less than 0.1 mass%, the ablation efficiency cannot be improved. If the content is more than 10 mass%, the hydrophilicity of the hydrophilic layer tends to droop.

### <Manufacture of the lithographic printing plate original>

To manufacture the lithographic printing plate original of the present invention, a coating solution containing at least a polymer with a pyrolytic group in the main chain and a crosslinking agent, which has the nonvolatile content adjusted to, preferably, 1-50 mass%, is coated on the surface of a support, which is then dried to form a lipophilic layer on the support.

When the lithographic printing plate original of the present has a hydrophilic layer, a coating solution containing at least a polymer for forming the hydrophilic layer, which has the nonvolatile content adjusted to, preferably, 1-50 mass%, is coated on the hydrophilic surface of a support, which is then dried to form a hydrophilic layer on the support. Then, a coating solution containing at least a polymer with a pyrolytic group in the main chain and a crosslinking agent is coated on the surface of the hydrophilic layer, which is then dried to form a lipophilic layer on the hydrophilic layer.

Conventional well-known organic solvents can be used for the coating solution. It is preferred to use an organic solvent with a boiling point in the range of 40-200°C, especially in the range of 60-160°C because it is desired for drying.

Examples of the organic solvents that can be used include methyl alcohol, ethyl alcohol, n- or iso-propyl alcohol, n- or iso-butyl alcohol, diacetone alcohol, and other alcohols; acetone, methyl ethyl ketone, methyl propyl ketone, methyl butyl ketone, methyl amyl ketone, methyl hexyl ketone, diethyl ketone, diisobutyl ketone, cyclohexanone, methyl cyclohexanone, acetyl acetone, and other ketones; hexane, cyclohexane, heptane, octane, nonane, decane, benzene, toluene, xylene, methoxybenzene, and other hydrocarbons; ethyl acetate, n- or iso-propyl acetate, n- or iso-butyl acetate, ethyl butyl acetate, hexyl acetate, and other acetates; methylene dichloride, ethylene dichloride, monochlorobenzene, and other halides; isopropyl ether, n-butyl ether, dioxane, dimethyl dioxane, tetrahydrofuran, and other ethers; ethylene glycol, methyl cellosolve, methyl cellosolve acetate, ethyl cellosolve, diethyl cellosolve, cellosolve acetate, butyl cellosolve, butyl cellosolve acetate, methoxy ethanol, diethylene glycol monomethyl ether, diethylene glycol dimethyl ether, diethylene glycol methyl ethyl ether, diethylene glycol diethyl ether, propylene glycol, propylene glycol monomethyl ether, propylene glycol monomethyl ether acetate, propylene glycol monoethyl ether, propylene glycol monoethyl ether acetate, propylene glycol monobutyl ether, 3-methyl-3-methoxybutanol, 1-methoxy-2-propanol, and other polyhydric alcohols and their derivatives; dimethyl sulfoxide, N,N-dimethyl formamide, methyl lactate, ethyl lactate, and other special solvents. These solvents can be used either alone or as a mixture of several types.

Examples of the coating methods that can be used include roll coating, dip coating, air knife coating, gravure coating, gravure offset coating, hopper coating, blade coating, wire doctor coating, spray coating, etc. The coating amount of the coating solution is preferred to be in the range of 10-100 mL/m².

The coating solution coated on the support or the hydrophilic layer is usually dried using heated air. It is preferred to perform heating in the range of 30-200°C, especially, 40-140°C. The drying temperature can be kept at a certain level or increased stepwise during drying.

In some cases, good results can also be obtained by using dry air to perform dehumidification. It is preferred to supply the heated air at a rate of 0.1-30 m/sec, especially, in the range of 0.5-20 m/sec to the coating surface.

The coating amount of the coating solution is usually in the range of 0.5-5 g/m² measured in dry mass.

### <Plate manufacturing method>

For the lithographic printing plate original of the present invention, direct plate manufacture is possible by irradiating an IR laser beam on the lipophilic layer based on the digital signals sent from a computer, etc.

The plate manufacturing method of the present invention is characterized by the fact that the lithographic printing plate of the present invention is exposed by the IR laser beam, and the lipophilic layer in the exposed part is pyrolyzed and removed.

A high output laser having maximum strength from the near IR region to the IR region is used as the IR laser beam light source in the present invention. More specifically, various types of lasers, such as a semiconductor laser and a YAG laser, having the is maximum strength from the near IR region to the IR region of 760-3000 nm, can be used.

Since the lithographic printing plate original of the present invention explained above has a lipophilic layer containing a crosslinked product generated when the polymer with a pyrolytic group in the main chain is crosslinked by a crosslinking agent, direct plate manufacture becomes possible by irradiating an IR laser beam based on digital signals. The plate can be directly loaded into a printer to carryout printing without performing development after exposure. In other words, when the lipophilic layer is exposed by the IR laser beam, the lipophilic layer in the exposed part is removed by the ablation induced by the laser to expose the support surface or the hydrophilic layer in the exposed part.

Also, since the lithographic printing plate original of the present invention has a polymer with pyrolytic group in the main chain, when the IR laser beam is irradiated, the pyrolytic groups are decomposed to cut off the main chain of the polymer. In this way, the ablation efficiency (sensitivity) can be improved significantly.

For the lithographic printing plate original of the present invention, since the polymer with a pyrolytic group in the main chain is crosslinked by the crosslinking agent, the printing durability of the lithographic printing plate obtained after the exposure treatment is excellent.

### Application Examples

In the following, the present invention will be explained in more detail with reference to application examples. The present invention, however, is not limited to these application examples. The nonvolatile content and the mass average molecular weight were measured using the following methods.

### [Measurement of the nonvolatile content]

About 1 g of sample was dried at 110°C in a dryer for 1 hour. The nonvolatile content was expressed in mass% based on the mass measurement conducted before and after the drying.

### [Measurement of the mass average molecular weight]

The mass average molecular weight was measured by means of gel penetration chromatography (GPC) and was expressed as polystyrene equivalent molecular weight.

The polymer with a pyrolytic group in the main chain was synthesized as follows.

### [Synthesis of polymer (P-1) containing azo groups]

212.4 g of dry N,N-dimethyl acetoamide, 128.8 g (100 mmol) of an azo compound represented by the following formula (a) [compound name: 2,2'-azobis(2-methyl-N-(2-(1-hydroxybutyl)propionamide)], and 28.8 g (100 mmol) of pyromellitic anhydride represented by the following formula (b) were add into a reaction container. While the mixture was stirred in the reaction container, 20.2 g (200 mmol) of triethyl amine was added dropwise as catalyst into the mixture in 1 h. The temperature of the reaction solution was raised to 40°C, and the color of the reaction solution changed from colorless to brown. After the catalyst was added, the mixture was stirred continuously for 10 h. Then, the solution containing the polymer (P-1) with a azo groups was removed. The nonvolatile content of the solution was 25 mass%. The mass average molecular weight of the azo containing polymer (P-1) was 4130.

### [Synthesis of azo containing polymer (P-2)]

138.4 g of dry N,N-dimethyl acetoamide, 14.4 g (50 mmol) of the azo compound represented by said formula (a), 25.02 g (100 mmol) of 4,4'-diphenyl methane diisocyanate represented by the following formula (c), and 6.71 g (50 mmol) of dimethylol propionic acid represented by the following formula (d) were added into a reaction container. While the mixture was stirred in the reaction container, 1 g of tin dibutyl dilaurate was added as catalyst into the mixture. The temperature of the reaction solution was raised to 35°C, and the viscosity of the reaction solution was increased. After the catalyst was added, the mixture was stirred continuously for 11 h. Then, the solution containing the azo containing polymer (P-2) was removed. The nonvolatile content of the solution was 25 mass%. The IR absorption spectrum was measured. It was confirmed that the absorption (2250-2275 cm⁻¹) typical of the isocyanate group disappeared. The mass average molecular weight of the azo containing polymer (P-2) was 7439.

### [Synthesis of azo containing polymer (P-3)]

243.6 g of dry N,N-dimethyl acetoamide, 20.0 g (100 mmol) of an azo compound represented by the following formula (e) [compound name: 2,2'-azobis(2-methyl-N-(2-hydroxyethylpropionamide)], and 41.0 g (100 mmol) of tetracarboxylic anhydride represented by the following formula (f) (TMEG-100, product of New Japan Rika Co., Ltd.) were added into a reaction container. While the mixture was stirred in the reaction container, 20.2 g (200 mmol) of triethyl amine was added dropwise as catalyst into the mixture in 1 h. The temperature of the reaction solution was raised to 43°C, and the color of the reaction solution changed from colorless to brown. After the catalyst was added, the mixture was stirred continuously for 10 h. Then, the solution containing the azo containing polymer (P-3) was removed. The nonvolatile content of the solution was 25 mass%. The mass average molecular weight of the azo containing polymer (P-3) was 6940.

### [Synthesis of ammonium containing polymer (P-4)]

11.9 g (100 mmol) of bis(2-hydroxyethyl)methyl amine and 15.61 g (110 mmol) of methyl iodide were added into a reaction container, followed by 2 h of reaction carried out at 90°C. Then, 300 mL of ethyl acetate was added into the reaction container, and the crystal generated was filtered out in a nitrogen atmosphere. The result of NMR analysis of the crystal obtained showed that the crystal was an ammonium containing compound represented by the following formula (g). The yield was 20 g.

204.3 g of dry N,N-dimethyl acetoamide, 26.1 g (100 mmol) of the ammonium containing compound represented by the following formula (g), and 21.8 g (100 mmol) of pyromellitic anhydride represented by said formula (b) were added into the reaction container. While the mixture was stirred in the reaction container, 20.2 g (200 mmol) of triethyl amine was added dropwise as catalyst into the mixture in 1 h. The temperature of the reaction solution was raised to 40°C, and the color of the reaction solution changed from colorless to brown. After the catalyst was added, the mixture was stirred continuously for 10 h. Then, the solution containing the ammonium polymer (P-4) was removed. The nonvolatile content of the solution was 25 mass%. The mass average molecular weight of the ammonium containing polymer (P-4) was 5630.

### [Synthesis of comparative polymer (P-5)]

166.2 g of dry N,N-dimethyl acetoamide, 13.4 g (100 mmol) of dimethylol propionic acid represented by said formula (d), and 21.8 g (100 mmol) of pyromellitic anhydride represented by said formula (b) were added into a reaction container. While the mixture was stirred in the reaction container, 20.2 g (200 mmol) of triethyl amine was added dropwise as catalyst into the mixture in 1 h. The temperature of the reaction solution was raised to 40°C, and the color of the reaction solution changed from colorless to brown. After the catalyst was added, the mixture was stirred continuously for 10 h. Then, the solution containing the comparative polymer (P-5) with no pyrolytic group in the main chain was removed. The nonvolatile content of the solution was 25 mass%. The mass average molecular weight of the polymer (P-5) was 3045.

### [Synthesis of azo containing polymer (P-6)]

131.8 g of dry N,N-dimethyl acetoamide, 4.4 g (50 mmol) of the azo compound represented by said formula (a), 25.02 g (100 mmol) of the 4,4'-diphenyl methane diisocyanate represented by said formula (c), and 4.51 g (50 mmol) of 2-methyl-1,3-propane diol represented by the following formula (h) were added into a reaction container. While the mixture was stirred in the reaction container, 1 g of tin diphenyl dilaurate was added as catalyst into the mixture. The temperature of the reaction solution was raised to 35°C, and the viscosity of the reaction solution was increased. After the catalyst was added, the mixture was stirred continuously for 11 h. Then, the solution containing the azo containing polymer (P-2) was removed. The nonvolatile content of the solution was 25 mass%. The IR absorption spectrum was measured. It was confirmed that the absorption (2250-2275 cm-1) typical to isocyanate group disappeared. The mass average molecular weight of the azo containing polymer (P-6) was 6851.

### [Aluminum support]

An aluminum sheet with a thickness of 0.24 mm was degreased using an aqueous solution of sodium hydroxide. The aluminum sheet was subjected to electrolytic polishing performed in a 20% hydrochloric acid bath to obtain a polished sheet with central line average roughness (Ra) of 0.5 µm. Then, the polished sheet was subjected to an anode oxidation treatment performed in a 20% sulfuric acid bath at a current density of 2A/dm² to form an oxidized film of 2.7 g/m². Then, the sheet was rinsed and dried to obtain an aluminum support.

### [Application Example 1]

7 g of polyvinyl alcohol (Poval 125, produced by Kuraray Co., Ltd.) was added into 140 g of deionized water. The mixture was stirred for 1 h while being heated at 100°C to dissolve the solid. After the system was cooled off, 10 g of an organic aluminum chelate compound (AL-135, product of Matsumoto Pharmaceutical Industrial Co., Ltd.) was added, followed by stirring to obtain a coating solution. The coating solution was coated by a #28 bar coater on the aluminum support, followed by 3 min of drying performed using 150°C hot air to form a hydrophilic layer (H-1) on the aluminum support. The dry coating film amount of the hydrophilic was 2.8 g/m².

30 g of the solution containing the azo containing polymer (P-1), 30 g of methyl cellosolve, 30 g of methyl ethyl ketone, 2 g of IR absorbing coloring material represented by the following formula (i) (IR-dyel [2(2-(2-chloro-3-((1,3-dihydro-1,1-dimethyl-3-(4-methyl)-2H-benzo (e) indole-2-ylidene)-1-ethylidene)-cyclohexene-1-yl)-ethenyl)-1,1-dimethyl-3-(4-methyl)-1H-benzo (e) indolium 4-toluene sulfonate], 2.5 g of hexamethoxymethyl melamine represented by the following formula (j) used as the crosslinking agent, and 0.1 g of BYK^{®}-333 (product of BYKCHEMICAL Corporation) used as surfactant were mixed to obtain a coating solution. The coating solution was coated with a #6 bar coater on the hydrophilic layer (H-1) to obtain a lithographic printing plate original. The dry coating film amount of the lipophilic layer was 1.0 g/m².

Image exposure was applied to the obtained lithographic printing plate original using an exposing device loaded with a near IR semiconductor laser (Trendsetter^{®}, product of Creo Corporation, wavelength 830 nm, laser power 15 W, rotation speed 96 rpm (equivalent to 375 mJ/cm²). The exposed part of the lipophilic layer was removed to expose the hydrophilic layer (H-1). The exposed part becomes hydrophilic, and it becomes the non-scanning part during printing. The exposed lithographic printing plate was set on a printer. After running idle several times on the printer, wetting water was applied from a dampening roller onto the lithographic printing plate. Then, printing was started. Ink was attached to the lipophilic layer in the non-exposed part. After 30000 copies were printed, the printing quality (stain, printing durability) was checked. The results are shown in Table 1.

### [Application Example 2]

7 g of polyvinyl alcohol (Poval 125, produced by Kuraray Co., Ltd.) was added into 140 g of deionized water. The mixture was stirred for I h while being heated at 100°C to dissolve the solid. Then, 10 g of an organic aluminum chelate compound (AL-135, product of Matsumoto Pharmaceutical Industrial Co., Ltd.) and 0.3 g of a water soluble IR absorbing coloring material represented by the following formula (k) (product of FEWCHEMICAL, 2-(2-(2-chloro-3-((1,3-dihydro-1,1-dimethyl-3-(4-sulfobutyl)-2H-benzo (e) indole-2-ylidene)-ethylidene)-1-cycylohexene-1-yl}ethenyl)-1,I-dimethyl-3-(4sulfobutyl}iH-benzo (e) indolium hydroxide, inner salt, sodium salt) were added, followed by stirring to obtain a coating solution. The coating solution was coated by a #28 bar coater on the aluminum support, followed by 3 min of drying performed using 150°C hot air to form a hydrophilic layer (H-2) on the aluminum support. The dry coating film amount of the hydrophilic was 2.8 g/m².

A lipophilic layer was formed on hydrophilic layer (H-2) in the same way as described in Application Example 1 to obtain a lithographic printing plate original. The dry coating film amount of the lipophilic layer was 1.0 g/m².

Then, image exposure was applied to the lithographic printing plate original obtained in the same way as described in Application Example 1. The exposed part of the lipophilic layer was removed to expose the hydrophilic layer (H-2). The exposed part becomes hydrophilic. It becomes the non-scanning part during printing. The exposed lithographic printing plate was set on a printer. After running idle several times on the printer, wetting water was applied from a dampening roller onto the lithographic printing plate. Then, printing was started. Ink was attached to the lipophilic layer in the non-exposed part. After 30000 copies were printed, the printing quality (stain, printing durability) was checked. The results are shown in Table 1.

### [Application Example 3]

7 g of polyvinyl alcohol (Poval 125, produced by Kuraray Co., Ltd.) was added into 140 g of deionized water. The mixture was stirred for 1 h while being heated at 100°C to dissolve the solid. Then, 10 g of an organic aluminum chelate compound (AL-135, product of Matsumoto Pharmaceutical Industrial Co., Ltd.) and 0.3 g of an aqueous carbon black (product of Cabot, Cabot Jet^{®} 300) were added, followed by stirring to obtain a coating solution. The coating solution was coated by a #28 bar coater on the aluminum support, followed by 3 min of drying performed using 150°C hot air to form a hydrophilic layer (H-3) on the aluminum support. The dry coating film amount of the hydrophilic layer was 2.8 g/m².

A lipophilic layer was formed on hydrophilic layer (H-3) in the same way as described in Application Example 1 to obtain a lithographic printing plate original. The dry coating film amount of the lipophilic layer was 1.0 g/m².

Then, image exposure was applied to the lithographic printing plate original obtained in the same way as described in Application Example 1. The exposed part of the lipophilic layer was removed to expose the hydrophilic layer (H-3). The exposed part becomes hydrophilic, and it becomes the non-scanning part during printing. The exposed lithographic printing plate was set on a printer. After running idle several times on the printer, wetting water was applied from a dampening roller onto the lithographic printing plate. Then, printing was started. Ink was attached to the lipophilic layer in the non-exposed part. After 30000 copies were printed, the printing quality (stain, printing durability) was checked. The results are shown in Table 1.

### [Application Example 4]

A lithographic printing plate original was manufactured in the same way as described in Application Example 1 except that the azo containing polymer (P-1) used for the lipophilic layer was changed to azo containing polymer (P-2). The dry coating film amount of the lipophilic layer was 1.0 g/m².

Then, image exposure was applied to the lithographic printing plate original obtained in the same way as described in Application Example 1. The exposed part of the lipophilic layer was removed to expose the hydrophilic layer (H-1). The exposed part becomes hydrophilic and it becomes the non-scanning part during printing. The exposed lithographic printing plate was set on a printer. After running idle several times on the printer, wetting water was applied from a dampening roller onto the lithographic printing plate. Then, printing was started. Ink was attached to the lipophilic layer in the non-exposed part. After 30000 copies were printed, the printing quality (stain, printing durability) was checked. The results are shown in Table 1.

### [Application Example 5]

A lithographic printing plate original was manufactured in the same way as described in Application Example 1 except that the azo containing polymer (P-1) used for the lipophilic layer was changed to azo containing polymer (P-3). The dry coating film amount of the lipophilic layer was 1.0 g/m².

Then, image exposure was applied to the lithographic printing plate obtained original in the same way as described in Application Example 1. The exposed part of the lipophilic layer was removed to expose the hydrophilic layer (H-1). The exposed part becomes hydrophilic, it becomes the non-scanning part during printing. The exposed lithographic printing plate was set on a printer. After running idle several times on the printer, wetting water was applied from a dampening roller onto the lithographic printing plate. Then, printing was started. Ink was attached to the lipophilic layer in the non-exposed part. After 30000 copies were printed, the printing quality (stain, printing durability) was checked. The results are shown in Table 1.

### [Application Example 6]

A lithographic printing plate original was manufactured in the same way as described in Application Example 1 except that the azo containing polymer (P-1) used for the lipophilic layer was changed to ammonium containing polymer (P-4). The dry coating film amount of the lipophilic layer was 1.0 g/m².

Then, image exposure was applied to the lithographic printing plate original obtained using an exposure device loaded with a near IR semiconductor laser (Trendsetter^{®}, product of Creo Corporation, wavelength 830 nm, laser power 15 W, rotation speed 72 rpm (equivalent to 500 mJ/cm2). The exposed part of the lipophilic layer was removed to expose the hydrophilic layer (H-1). The exposed part becomes hydrophilic, and it becomes the non-scanning part during printing. The exposed lithographic printing plate was set on a printer. After running idle several times on the printer, wetting water was applied from a dampening roller onto the lithographic printing plate. Then, printing was started. Ink was attached to the lipophilic layer in the non-exposed part. After 30000 copies were printed, the printing quality (stain, printing durability) was checked. The results are shown in Table 1.

### [Application Example 7]

A lithographic printing plate original was manufactured in the same way as described in Application Example 1 except that the azo containing polymer (P-1) used for the lipophilic layer was changed to azo containing polymer (P-6). The dry coating film amount of the lipophilic layer was 1.0 g/m².

Then, image exposure was applied to the lithographic printing plate original obtained using an exposure device loaded with a near IR semiconductor laser (Trendsetter^{®}, product of Creo Corporation, wavelength 830 nm, laser power 15 W, rotation speed 180 rpm (equivalent to 200 mJ/cm²). The exposed part of the lipophilic layer was removed to expose the hydrophilic layer (H-1). The exposed part becomes hydrophilic, and it becomes the non-scanning part during printing. The exposed lithographic printing plate was set on a printer. After running idle several times on the printer, wetting water was applied from a dampening roller onto the lithographic printing plate. Then, printing was started. Ink was attached to the lipophilic layer in the non-exposed part. After 30000 copies were printed, the printing quality (stain, printing durability) was checked. The results are shown in Table 1.

### [Comparative Example 1]

A lithographic printing plate original was manufactured in the same way as described in Application Example 1 except that the azo containing polymer (P-1) used for the lipophilic layer was changed to comparative polymer (P-5). The dry coating film amount of the lipophilic layer was 1.0 g/m².

Then, image exposure was applied to the lithographic printing plate original obtained in the same way as described in Application Example 1. The exposed part of the lipophilic layer was not removed and left as it was.

**Table 1**

| | Polymer of the lipophilic layer | Hydrophilic layer | Sensitivity | Printing durability | Printing quality |
|---|---|---|---|---|---|
| Application Example 1 | P-1 | H-1 | Good | Good | Good |
| Application Example 2 | P-1 | H-2 | Good | Good | Good |
| Application Example 3 | P-1 | H-3 | Good | Good | Good |
| Application Example 4 | P-2 | H-1 | Good | Good | Good |
| Application Example 5 | P-3 | H-1 | Good | Good | Good |
| Application Example 6 | P-4 | H-1 | Slow | Good | Stain |
| Application Example 7 | P-6 | H-1 | Very fast | Poor | Good |
| Comparative Example 1 | P-5 | H-1 | Poor exposure | - | - |

In Table 1, good "sensitivity" means that the lipophilic layer can be completely removed even using a low output laser beam. "Slow" means that a high output laser beam is needed to completely remove the lipophilic layer.

For the lithographic printing plate originals obtained in Application Examples 1-7 using polymers with a pyrolytic group in the main chain, the lipophilic layer in the exposed part can be removed by the exposure treatment, and printing can be performed directly without carrying out development.

The lithographic printing plate originals of Application Examples 1-5, 7 using the azo containing polymers that can generate gas during pyrolysis have good sensitivity (ablation efficiency).

Also, the lithographic printing plate originals obtained in Application Examples 1-6 having functional groups in the polymer that can crosslink with the crosslinking agent have good printing durability.

### Industrial application possibility

The lithographic printing plate original of the present invention can be manufactured directly by irradiating an IR laser beam based on digital signals. The plate obtained can be loaded directly into a printer to perform printing without carrying out development after exposure. The ablation efficiency (sensitivity) is good, and the printing durability of the lithographic printing plate obtained is excellent. By using the aforementioned lithographic printing plate original, the plate manufacturing process can be simplified, and the operating environment of the plate manufacturing site can be improved. The adverse effect on the environment can also be reduced.

## Claims

1. A lithographic printing plate original wherein the lithographic printing plate original has a support having a hydrophilic surface and a lipophilic layer formed on that support,
the lipophilic layer contains a crosslinked product generated when a polymer with a pyrolytic group in the main chain is crosslinked by a crosslinking agent wherein the pyrolytic group is an azo, diazo, hydrazide, nitro, or ammonium salt.

2. The lithographic printing plate original according to Claim 1 **characterized by** the fact that the aforementioned pyrolytic group is azo group.

3. The lithographic printing plate original according to Claim I **characterized by** the fact that the aforementioned polymer has functional groups that can react with the crosslinking agent

4. The lithographic printing plate original according to any of Claims 1-3 **characterized by** the fact that the aforementioned lipophilic layer contains a light-heat converting substance.

5. The lithographic printing plate original according to any of Claims 1-4 **characterized by** the fact that there is a hydrophilic layer between the aforementioned support and the lipophilic layer.

6. The lithographic printing plate original according to Claim 5 **characterized by** the fact that the aforementioned hydrophilic layer contains a light-heat converting substance.

7. A plate manufacturing method **characterized by** the fact that the lithographic printing plate original according to any of Claims 1-6 is exposed by using an IR laser beam to remove the lipophilic layer in the exposed part.

## Patentansprüche

1. Offsetdruckplattenoriginal, worin das Offsetdruckplattenoriginal einen Träger mit einer hydrophilen Oberfläche und einer auf dem Träger ausgebildeten lipophilen Schicht aufweist,
wobei die lipophile Schicht ein vernetztes Produkt enthält, das erzeugt wird, wenn ein Polymer mit einer pyrolytischen Gruppe in der Hauptkette von einem Vernetzungsmittel vernetzt wird, worin die pyrolytische Gruppe ein Azo-, Diazo-, Hydrazid-, Nitro- oder Ammoniumsalz ist.

2. Offsetdruckplattenoriginal nach Anspruch 1, **dadurch gekennzeichnet, dass** die zuvor genannte pyrolytische Gruppe eine Azogruppe ist.

3. Offsetdruckplattenoriginal nach Anspruch 1, **dadurch gekennzeichnet, dass** das zuvor genannte Polymer Funktionsgruppen aufweist, die mit dem Vernetzungsmittel zu reagieren vermögen.

4. Offsetdruckplattenoriginal nach einem der Ansprüche 1-3, **dadurch gekennzeichnet, dass** die zuvor genannte Offsetschicht einen Licht-Wärme-Umwandlungsstoff enthält.

5. Offsetdruckplattenoriginal nach einem der Ansprüche 1-4, **dadurch gekennzeichnet, dass** zwischen dem zuvor genannten Träger und der lipophilen Schicht eine hydrophile Schicht angeordnet ist.

6. Offsetdruckplattenoriginal nach Anspruch 5, **dadurch gekennzeichnet, dass** die zuvor genannte hydrophile Schicht einen Licht-Wärme-Umwandlungsstoff enthält.

7. Plattenherstellungsverfahren, **dadurch gekennzeichnet, dass** das Offsetdruckplattenoriginal nach einem der Ansprüche 1-6 mit einem Infrarot-Laserstrahl belichtet wird, um die lipophile Schicht in dem belichteten Bereich zu entfernen.

## Revendications

1. Original de plaque d'impression lithographique dans lequel l'original de la plaque d'impression lithographique comprend un support revêtu d'une surface hydrophile et d'une couche lipophile,
la couche lipophile contient un produit réticulé généré lorsqu'un polymère contenant un groupe pyrolytique dans la chaîne principale est réticulé par un agent de réticulation, dans lequel le groupe pyrolytique est un sel azo, diazo, hydrazide, nitro ou ammonium.

2. Original de plaque d'impression lithographique selon la revendication 1, **caractérisé par le fait que** le groupe pyrolytique précédemment mentionné est un groupe azo.

3. Original de plaque d'impression lithographique selon la revendication 1, **caractérisé par le fait que** le polymère précédemment mentionné contient des groupes fonctionnels pouvant réagir avec l'agent de réticulation.

4. Original de plaque d'impression lithographique selon l'une quelconque des revendications 1 à 3, **caractérisé par le fait que** la couche lipophile précédemment mentionnée contient une substance de conversion de la lumière en chaleur.

5. Original de plaque d'impression lithographique selon l'une quelconque des revendications 1 à 4, **caractérisé par le fait qu'**une couche hydrophile se trouve entre le support précédemment mentionné et la couche lipophile.

6. Original de plaque d'impression lithographique selon la revendication 5, **caractérisé par le fait que** la couche hydrophile précédemment mentionnée contient une substance de conversion de la lumière en chaleur.

7. Procédé de fabrication de plaque **caractérisé par le fait que** l'original de la plaque d'impression lithographique selon l'une quelconque des revendications 1 à 6 est exposé en utilisant un faisceau laser IR pour éliminer la couche lipophile dans la partie exposée.
